



US005863686A

# United States Patent [19]

Yuh et al.

[11] Patent Number: **5,863,686**[45] Date of Patent: **Jan. 26, 1999**

[54] **PHOTORECEPTOR WITH DONOR MOLECULE IN CHARGE GENERATING LAYER**

[75] Inventors: **Huoy-Jen Yuh**, Pittsford; **John S. Chambers**, Rochester; **Damodar M. Pai**, Fairport; **John F. Yanus**, Webster, all of N.Y.

[73] Assignee: **Xerox Corporation**, Stamford, Conn.

[21] Appl. No.: **4,268**

[22] Filed: **Jan. 8, 1998**

[51] Int. Cl.<sup>6</sup> ..... **G03G 5/047**; G03G 5/09

[52] U.S. Cl. ..... **430/59**; 430/58; 430/83; 430/134

[58] Field of Search ..... 430/58, 59, 83, 430/134

## [56] References Cited

### U.S. PATENT DOCUMENTS

4,588,666 5/1986 Stolka et al. ..... 430/59

4,871,634 10/1989 Limburg et al. ..... 430/54  
5,011,939 4/1991 Limburg et al. ..... 548/440  
5,342,719 8/1994 Pai et al. ..... 430/59  
5,436,099 7/1995 Schank et al. ..... 430/59

Primary Examiner—Roland Martin

## [57] ABSTRACT

An electrophotographic imaging member comprising a supporting substrate, an undercoat layer doped with an donor molecule a charge generating layer comprising photoconductive pigment particles, film forming binder and an donor molecule dissolved in the film forming binder, and a charge transport layer,

the charge generating layer being located between the substrate and the charge transport layer. A process for fabricating this imaging member is also disclosed.

**10 Claims, No Drawings**

**PHOTORECEPTOR WITH DONOR  
MOLECULE IN CHARGE GENERATING  
LAYER**

**BACKGROUND OF THE INVENTION**

This invention relates in general to electrophotography and more specifically, to an improved electrophotographic imaging member having an a more sensitive charge generating layer.

In the art of electrophotography, an electrophotographic plate comprising a photoconductive insulating layer on a conductive layer is imaged by first uniformly electrostatically charging surface of the photoconductive insulating layer. The plate is then exposed to a pattern of activating electromagnetic radiation such as light, which selectively dissipates the charge in the illuminated areas of the photoconductive insulating layer while leaving behind an electrostatic latent image in the non-illuminated areas. This electrostatic latent image may then be developed to form a visible image by depositing finely divided electroscopic toner particles on the surface of the photoconductive insulating layer. The resulting visible toner image can be transferred to a suitable receiving member such as paper. This imaging process may be repeated many times with reusable photoconductive insulating layers.

Electrophotographic imaging members are usually multilayered photoreceptors that comprise a substrate support, an electrically conductive layer, an optional hole blocking layer, an adhesive layer, a charge generating layer, and a charge transport layer in either a flexible belt form or a rigid drum configuration. For most multilayered flexible photoreceptor belts, an anti-curl layer is usually employed on the back side of the substrate support, opposite to the side of the electrically active layers, to render the desired photoreceptor flatness. One type of multilayered photoreceptor comprises a layer of finely divided particles of a photoconductive inorganic compound dispersed in an electrically insulating organic resin binder. In U.S. Pat. No. 4,265,990 a layered photoreceptor is disclosed having separate charge generating (photogenerating) and charge transport layers. The charge generating layer is capable of photogenerating holes and injecting the photogenerated holes into the charge transport layer. The photogenerating layer utilized in multilayered photoreceptors include, for example, inorganic photoconductive particles or organic photoconductive particles dispersed in a film forming polymeric binder. Inorganic or organic photoconductive material may be formed as a continuous, homogeneous photogenerating layer. Many suitable photogenerating materials known in the art can be utilized, if desired.

As more advanced, higher speed electrophotographic copiers, duplicators and printers were developed, degradation of image quality was encountered during extended cycling. Moreover, complex, highly sophisticated, duplicating and printing systems employed flexible photoreceptor belts, operating at very high speeds, have also placed stringent mechanical requirements and narrow operating limits as well on photoreceptors. Advanced photoreceptors have excellent electrical and mechanical properties. Some have very stable electrical performance over long life, for example, up to at least 200K cycles. However, many photoreceptors exhibit fluctuations in photosensitivity from batch to batch even where every effort is made to ensure identical processing conditions such as the milling of charge generation layer pigment dispersion under the same conditions. For example, when extrinsic photosensitive pigments

are employed, the photogenerated carriers must be brought out of the surface of pigment particles before the carriers recombine and move into the charge transport layer under the applied electric field. This process slows down considerably in binders containing dispersed extrinsic photosensitive pigment particles such as benzimidazole perylene particles, especially at low applied electric fields. Under these conditions, the photoinduced discharged curve (PIDC) becomes softer at low field. Such a soft PIDC curve requires more powerful, bulky and expensive laser light sources for imaging in an electrophotographic printer or duplicator. The expression photoinduced discharged curve (PIDC) as employed herein is defined as a relationship between the potential as a function of exposure and is a measure of the sensitivity of the device. It generally represents the supply efficiency (number carriers injected from the generator layer into the transport layer per incident photon) as a function of the field across the device.

**INFORMATION DISCLOSURE STATEMENT**

U.S. Pat. No. 4,871,634 to Limburg et al., issued Oct. 3, 1989—A hydroxy arylamine compound is disclosed represented by specific formula; the dihydroxy arylamine compound being free of any direct conjugation between the —OH groups and the nearest nitrogen atom through one or more aromatic rings. The dihydroxy arylamine compound may be employed in an electrophotographic imaging member and the member may be used in an electrophotographic imaging process. This hydroxy arylamine may be used with a polar resin in the charge generator layer.

U.S. Pat. No. 5,011,939 to Limburg et al., issued Apr. 30, 1991—A hydroxy arylamine compound is disclosed as described in parent patent U.S. Pat. No. 4,871,634 above.

U.S. Pat. No. 4,588,666 to Stolka et al., issued May 13, 1986—A hole transporting molecule comprised of alkoxy derivatives of tetra phenyl biphenyl diamine represented by a specified formula and layered imaging members containing therein the aforementioned alkoxydiamine derivatives and a photoconductive layer are disclosed.

U.S. Pat. No. 5,342,719 issued to Pai et al. on Aug. 30, 1994—An electrophotographic imaging member is disclosed including a charge generator layer, a charge transport layer with charge transport molecules and as sensitizing additive or dopant a hydroxy derivative of the transport molecule.

Thus, there is a continuing need for photoreceptors having improved sensitivity, and for tools or control techniques to adjust the sensitivity of an electrophotographic imaging device to meet stringent specifications in spite of the batch to batch variations in the quality of the various materials employed to fabricate the generator layer, undercoating layer and transport layers, especially the pigment.

**CROSS REFERENCE TO COPENDING  
APPLICATIONS**

Application Ser. No. 09/004,269 filed in the names of Yuh et al., entitled PHOTORECEPTOR WITH IMPROVED CHARGE GENERATING LAYER, filed concurrently herewith Jan. 8, 1998 (Attorney Docket No. D/97388)—An electrophotographic imaging member is disclosed comprising a supporting substrate, an undercoat layer, a charge generating layer comprising photoconductive pigment particles, film forming binder and an acceptor molecule dissolved in the film forming binder, and a charge transport layer, the charge generating layer being located between the substrate and the charge transport layer. A process for fabricating this imaging member is also disclosed.

## BRIEF SUMMARY OF THE INVENTION

It is, therefore, an object of the present invention to provide an improved electrophotographic imaging member and process for fabricating the imaging member.

It is another object of the present invention to provide an improved electrophotographic imaging member having greater sensitivity.

It is still another object of the present invention to provide an improved electrophotographic imaging member in which diffusion of dopant from the charge generating layer to the charge transport layer is reduced.

It is yet another object of the present invention to provide a quality control tool or device to precisely control the sensitivity of an electrophotographic imaging member within high tolerance specifications in spite of quality variations between component material batches, especially pigments.

It is another object of the present invention to provide a quality control tool or device to precisely control the sensitivity of an electrophotographic imaging member within high tolerance specifications without major changes in the dispersion quality of the generator layer solutions or without any major changes to the fabrication process of the member.

The foregoing objects and others are accomplished in accordance with this invention by providing an electrophotographic imaging member comprising

- a supporting substrate,
- an undercoat layer,
- a charge generating layer comprising
  - photoconductive pigment particles selected from the group consisting of benzimidazole perylene and dibromoanthanthrone,
  - a film forming binder of polyvinyl butyral, and
  - a donor charge transporting molecule dissolved in the binder, the donor charge transport molecule selected from the group consisting of N,N'-diphenyl-N,N'-bis(3-hydroxyphenyl)-[1,1'-biphenyl]-4,4'-diamine, N,N'-di(3-methoxyphenyl)-N,N'-diphenyl-[1,1'-biphenyl]-4,4'-diamine and mixtures thereof and
- a charge transport layer,
- the charge generating layer being located between the substrate and the charge transport layer.

This imaging member may be fabricated by

- forming a charge generating layer from a coating solution of comprising
  - photoconductive pigment selected from the group consisting of particles of benzimidazole perylene and dibromoanthanthrone dispersed in a film forming binder of polyvinyl butyral,
  - a hole transporting small molecule selected from the group consisting of N,N'-diphenyl-N,N'-bis(3-hydroxyphenyl)-[1,1'-biphenyl]-4,4'-diamine, or N,N'-di(3-methoxyphenyl)-N,N'-diphenyl-[1,1'-biphenyl]-4,4'-diamine and mixtures thereof dissolved in the binder,
- forming a charge transport layer coating comprising
  - N,N'-diphenyl-N,N'-bis(3-methylphenyl)-[1,1'-biphenyl]-4,4'-diamine and
  - a polycarbonate binder and
  - a solvent mixture of monochlorobenzene and tetrahydrofuran,
- drying the coating to form a charge transport layer overlying the charge generating layer.

Generally, electrophotographic imaging members comprise a supporting substrate, having an electrically conduc-

tive surface or coated with an electrically conductive layer, an optional charge blocking layer, an undercoat layer, a charge generating layer, a charge transport layer and an optional overcoating layer.

- 5 The substrate may be opaque or substantially transparent and may comprise numerous suitable materials having the required mechanical properties. Accordingly, this substrate may comprise a layer of an electrically non-conductive or conductive material such as an inorganic or an organic composition. The electrically conductive layer may comprise the entire supporting substrate or merely be present as a coating on an underlying rigid or flexible web member. Any suitable electrically conductive material may be utilized. Typical electrically conductive materials include, for example, aluminum, titanium, nickel, chromium, brass, gold, stainless steel, copper iodide, and the like. When the conductive layer is to be flexible, it may vary in thickness over substantially wide ranges depending on the desired use of the electrophotocuctive member. Accordingly, the conductive layer can generally range in thicknesses of from about 50 Angstrom units to about 150 micrometers. As electrically non-conducting materials there may be employed various thermoplastic and thermoset resins known for this purpose including polyesters, polycarbonates, polyamides, polyurethanes, and the like. The substrate may have any suitable shape such as, for example, a flexible web, rigid cylinder, sheet and the like.

The thickness of a flexible substrate support depends on numerous factors, including economical considerations, and thus this layer for a flexible belt may be of substantial thickness, for example, over 200 micrometers, or of minimum thickness less than 50 micrometers, provided there are no adverse affects on the final photoconductive device.

- 50 Any suitable hole blocking layer capable of forming an electronic barrier to holes between the adjacent photoconductive layer and the underlying conductive layer may be utilized. A hole blocking layer may comprise any suitable material. Typical hole blocking layers utilized for the negatively charged photoreceptors may include, for example, Luckamide, hydroxy alkyl methacrylates, nylons, gelatin, hydroxyl alkyl cellulose, organopolypophazines, organosilanes, organotitanates, organozirconates, silicon oxides, zirconium oxides, and the like. Preferably, the hole blocking layer comprises nitrogen containing siloxanes. Typical nitrogen containing siloxanes are prepared from coating solutions containing a hydrolyzed silane. Typical hydrolyzable silanes include 3-aminopropyl triethoxysilane, (N,N'-dimethyl 3-amino) propyl triethoxysilane, N,N-dimethylamino phenyl triethoxy silane, N-phenyl aminopropyl trimethoxy silane, trimethoxy silylpropylidene triamine and mixtures thereof.

During hydrolysis of the amino silanes described above, the alkoxy groups are replaced with hydroxyl group. An especially preferred blocking layer comprises a reaction product between a hydrolyzed silane and the oxidized surface of an underlying conductive layer which inherently forms on the surface of conductive a metal layer when exposed to air after deposition. This combination reduces spots at time 0 and provides electrical stability at low RH.

- 60 The imaging member is prepared by depositing on the conductive layer of a coating of an aqueous solution of the hydrolyzed silane at a pH between about 4 and about 10, drying the reaction product layer to form a siloxane film and applying electrically active layers, such as a photogenerator layer and a hole transport layer, to the siloxane film.

The blocking layer may be applied by any suitable conventional technique such as spraying, dip coating, draw

bar coating, gravure coating, silk screening, air knife coating, reverse roll coating, vacuum deposition, chemical treatment and the like. For convenience in obtaining thin layers, the blocking layers are preferably applied in the form of a dilute solution, with the solvent being removed after deposition of the coating by conventional techniques such as by vacuum, heating and the like. This siloxane coating is described in U.S. Pat. No. 4,464,450, the disclosure of thereof being incorporated herein in its entirety. After drying, the siloxane reaction product film formed from the hydrolyzed silane contains larger molecules. The reaction product of the hydrolyzed silane may be linear, partially crosslinked, a dimer, a trimer, and the like.

A preferred charge blocking layer may be fabricated from a solution of zirconium butoxide and gamma-amino propyl tri-methoxy silane in a suitable solvent such as an isopropyl alcohol, butyl alcohol and water mixture. Generally, a preferred solution comprises between about 70 and about 90 by weight of zirconium butoxide and between about 30 and about 10 by weight of gamma-amino propyl tri-methoxy silane, based on the total weight of solids in the solution.

The blocking layer should be continuous and have a thickness of less than about 0.5 micrometer because greater thicknesses may lead to undesirably high residual voltage. A blocking layer of between about 0.005 micrometer and about 0.3 micrometer (50 Angstroms-3000 Angstroms) is preferred because charge neutralization after the exposure step is facilitated and optimum electrical performance is achieved. A thickness of between about 0.03 micrometer and about 0.06 micrometer is preferred for metal oxide layers for optimum electrical characteristics.

Any suitable undercoat layer may be applied to the charge blocking layer. Undercoat layer materials are well known in the art. Typical undercoat layer materials include, for example, polyesters, MOR-ESTER 49,000 (available from Morton International Inc.), Vitel PE-100, Vitel PE-200, Vitel PE-200D, and Vitel PE-222 (all Vitels available from Goodyear Tire and Rubber Co.), polyarylates (Ardel, available from AMOCO Production Products), polysulfone (available from AMOCO Production Products), polyurethanes, and the like. The MOR-ESTER 49000 polyester resin is a linear saturated copolyester reaction product of ethylene glycol with terephthalic acid, isophthalic acid, adipic acid and azelaic acid. Other polyester resins which are chemically similar to the 49000 polyester resin and which are also suitable for a photoreceptor undercoat layer coating include Vitel PE-100 and Vitel PE-200, both of which are available from Goodyear Tire & Rubber Co. An especially preferred undercoat layer material is a polyamide such as Luckamide 5003 from Dai Nippon Ink, Nylon 8 with methylmethoxy pendant groups, CM 4000 and CM 8000 from Toray Industries Ltd and other N-methoxymethylated polyamides, such as those prepared according to the method described in Sorenson and Campbell "Preparative Methods of Polymer Chemistry", second edition, pg 76, John Wiley and Sons Inc. 1968, and the like and the mixtures thereof. These polyamides can be alcohol soluble, for example, with polar functional groups, such as methoxy, ethoxy and hydroxy groups, pendant from the polymer backbone. Any suitable alcohol solvent or solvent mixtures may be employed to form a coating solution. Typical solvents include methanol, ethanol, propanol and mixtures thereof. Water may optionally be added to the solvent mixture. Satisfactory results may be achieved with a dry undercoat layer thickness between about 0.05 micrometer and about 0.3 micrometer. Conventional techniques for applying an undercoat layer coating mixture to the charge blocking layer include spraying, dip

coating, roll coating, wire wound rod coating, gravure coating, Bird applicator coating, and the like. Drying of the deposited coating may be effected by any suitable conventional technique such as oven drying, infra red radiation drying, air drying and the like.

In some embodiments, the undercoat layer functions as a blocking layer and there is no need for a separate blocking layer underneath the undercoat layer.

Any suitable charge generating binder layer materials comprising photoconductive particles dispersed in a film forming binder may be utilized in combination with a hole transporting small molecule selected from the group consisting of N, N'-diphenyl-N,N'bis(3-hydroxyphenyl)-[1,1'-biphenyl]-4,4' diamine, or N,N'-di(3-methoxyphenyl)-N, 15 N'diphenyl-[1,1-biphenyl]-4,4'-diamine and mixtures thereof dissolved in the binder. Photoconductive particles for charge generating binder layer are selected from the group consisting of benzimidazole perylene and dibromoanthanthrone. Benzimidazole perylene and dibromoanthanthrone are known photoconductive materials.

The polymeric film forming binder material employed as the matrix in the charge generating (charge generation) binder layer is polyvinyl butyral. Preferably, the polyvinyl butyral is a film forming polymer having a polyvinyl butyral content between about 50 and about 75 mol percent, a polyvinyl alcohol content between about 12 and about 50 mol percent, and a polyvinyl acetate content is between about 0 to 15 mol percent. This polyvinyl is described in U.S. Pat. No. 5,418,107, the entire disclosure thereof being incorporated herein by reference.

Any suitable organic solvent may be utilized to dissolve the film forming binder. Typical solvents include n-butyl acetate, cyclohexanone, methyl ethyl ketone (MEK) and the like. The solvent n-butyl acetate is preferred because the dispersion quality of the coating mixture is superior. Coating dispersions for charge generating layer may be formed by any suitable technique using, for example, attritors, ball mills, Dynomills, paint shakers, homogenizers, microfluidizers, and the like.

The charge generation layer containing photoconductive pigments and the resinous binder material generally has a thickness of between about 0.1 micrometer and about 5 micrometers, and preferably has a thickness of between about 0.3 micrometer and about 2 micrometers. The charge generation layer thickness is related to binder content. Higher binder content compositions generally require thicker layers for photogeneration. Thicknesses outside these ranges can be selected providing the objectives of the present invention are achieved. Typical charge generating layer thicknesses have an optical density of between about 1.7 and about 2.1.

Any suitable and conventional technique may be utilized to mix and thereafter apply the charge generation layer coating mixture. Typical application techniques include slot coating, gravure coating, roll coating, spray coating, spring wound bar coating, dip coating, draw bar coating, reverse roll coating, and the like.

Any suitable drying technique may be utilized to solidify and dry the deposited coatings. Typical drying techniques include oven drying, forced air drying, infrared radiation drying, and the like.

The charge generation composition or pigment is present in the resinous binder composition in various amounts. Generally, however, from about 5 percent by volume to about 90 percent by volume of the charge generation pigment is dispersed in about 10 percent by volume to about 95 percent by volume of the resinous binder, and preferably

from about 20 percent by volume to about 30 percent by volume of the charge generation pigment is dispersed in about 70 percent by volume to about 80 percent by volume of the resinous binder composition.

As indicated above, the charge generating layer of the photoreceptor of this invention preferably comprises a perylene or dibromo anthanthrone pigment as a solution coated layer containing the pigment dispersed in a film forming resin binder. For photoreceptors utilizing a perylene charge generating layer, the perylene pigment is preferably benzimidazole perylene which is also referred to as bis (benzimidazole). This pigment exists in the cis and trans forms. The cis form is also called bis-benzimidazo(2,1-a'1', 1'-b) anthra (2,1,9-def:6,5,10-d'e'f) disoquinoline-6,11-dione. The trans form is also called bisbenzimidazo (2,1-a'1',1'-b) anthra (2,1,9-def:6,5,10-d'e'f) disoquinoline-10,21-dione. This pigment may be prepared by reacting perylene 3,4,9,10-tetracarboxylic acid dianhydride with 1,2-phenylene. Benzimidazole perylene compositions are well known and described, for example, in U.S. Pat. No. 5,019,473 and U.S. Pat. No. 4,587,189, the entire disclosures thereof being incorporated herein by reference. Benzimidazole perylene may be ground into fine particles having an average particle size of less than about 1 micrometer. Optimum results are achieved with a pigment particle size between about 0.2 micrometer and about 0.3 micrometer. Other suitable charge generation materials known in the art may also be utilized, if desired.

Photoreceptor embodiments prepared with a charge generating layer comprising benzimidazole perylene or dibromoanthanthrone dispersed in various types of resin binders give very poor dispersions, but the sensitivity of these photoreceptors have been found to be dramatically improved, particularly, with the use of benzimidazole perylene dispersed in polyvinyl butyral in combination with the donor molecule dissolved in the polyvinyl butyral film forming binder. Also, the dispersion quality of this combination of benzimidazole perylene, polyvinyl butyral, and donor molecule is superior.

The expression donor molecule, as employed herein, is defined as a molecule that donates an electron to the pigment especially when it is exposed to light and an exciton is created within it. The exciton is a hole-electron pair that are still attracted to each other and move as a pair. Typical donor molecules include, for example, triphenylmethane, bis(4-diethylamine-2-methylphenyl)phenylmethane; 4'-4"-bis(diethylamino)-2',2"-dimethyltriphenylmethane, N,N'-bis(alkylphenyl)-[1,1'-biphenyl]-4,4'-diamine wherein the alkyl is, for example, methyl, ethyl, propyl, n-butyl, etc., N,N'-diphenyl-N,N'-bis(chlorophenyl)-[1,1'-biphenyl]-4,4'-diamine, N,N'-diphenyl-N,N'-bis(3"-methylphenyl)-(1,1'-biphenyl)-4,4'-diamine, and the like. Preferred donor molecules are those selected from the group consisting of N,N'-diphenyl-N,N'-bis(3-hydroxyphenyl)-[1,1'-biphenyl]-4,4'-diamine, N,N'-di(3-methoxyphenyl)-N,N'-diphenyl-[1,1'-biphenyl]-4,4'-diamine and mixtures thereof. N,N'-diphenyl-N,N'-bis(3-hydroxyphenyl)-[1,1'-biphenyl]-4,4'-diamine is a known material which is disclosed, for example in U.S. Pat. No. 4,871,634 and U.S. Pat. No. 5,011,939, the entire disclosures of these two patents being incorporated herein by reference. N,N'-di(3-methoxyphenyl)-N,N'-diphenyl-[1,1'-biphenyl]-4,4'-diamine is also a known material which is disclosed, for example in U.S. Pat. No. 4,871,634, U.S. Pat. No. 5,011,939 and U.S. Pat. No. 4,588,666 the entire disclosures of these three patents being incorporated herein by reference.

Satisfactory results are achieved when the dried charge generating layer of the final imaging member contains

between about 5 and about 30 percent by weight of donor molecule, based on the total weight of the charge generating layer. When the proportion of donor molecule is less than about 1 percent by weight, based on the total weight of the charge generating layer, the imaging member shows no improvement in the sensitivity. When the proportion of acceptor is greater than about 40 percent by weight, based on the total weight of the charge generating layer, the imaging member phase separation may occur resulting in undesirable cyclic stability issues such as residual cycle-up. Preferably, the dried charge generating layer of the final imaging member contains between about 5 and about 30 percent by weight of donor molecule, based on the total weight of the charge generating layer.

A donor molecule is deemed soluble in the specific solvent and the specific film forming binder used in the charge generating layer when a clear, transparent solution is formed by the mixture of the three miscible components. The donor molecule should also be insoluble in the solvent and film forming binder used for the undercoat. In addition, the film forming binder used in the undercoat layer should be insoluble in the solvent used for the charge generating layer. Further, the film forming binder used in the undercoat layer should not be miscible with the film forming binder in the charge generating layer. Illustrative combinations of miscible donor molecules and film forming binders for the charge generating layer include, for example, polyvinyl butyral (PVB) and N,N'-diphenyl-N,N'-bis(3-hydroxyphenyl)-[1,1'-biphenyl]-4,4'-diamine, polyvinyl butyral and N,N'-di(3-methoxyphenyl)-N,N'-diphenyl-[1,1'-biphenyl]-4,4'-diamine, polyvinyl butyral and N,N'-diphenyl-N,N'-bis(3-hydroxyphenyl)-[1,1'-biphenyl]-4,4'-diamine, polyvinyl butyral and N,N'-di(3-methoxyphenyl)-N,N'-diphenyl-[1,1'-biphenyl]-4,4'-diamine, and the like.

Any suitable charge transport layer may be utilized on the charge generator layer. The active charge transport layer may comprise any suitable transparent organic polymer of non-polymeric material capable of supporting the injection of photo-generated holes and electrons from the charge generating layer and allowing the transport of these holes or electrons through the organic layer to selectively discharge the surface charge. The charge transport layer in conjunction with the generation layer in the instant invention is a material which is an insulator to the extent that an electrostatic charge placed on the transport layer is not conducted in the absence of illumination. Thus, the active charge transport layer is a substantially non-photoconductive material which supports the injection of photogenerated holes from the generation layer.

An especially preferred transport layer employed in one of the two electrically operative layers in the multilayer photoconductor of this invention comprises from about 25 to about 75 percent by weight of at least one charge transporting aromatic amine compound, and about 75 to about 25 percent by weight of a polymeric film forming resin in which the aromatic amine is soluble. A dried charge transport layer containing between about 40 percent and about 50 percent by weight of the small molecule charge transport molecule based on the total weight of the dried charge transport layer is preferred.

The charge transport layer forming mixture preferably comprises an aromatic amine compound. Typical aromatic amine compounds include triphenyl amines, bis and poly triarylamines, bis arylamine ethers, bis alkyl-aryl amines and the like.

Examples of charge transporting aromatic amines for charge transport layers capable of supporting the injection of

photogenerated holes of a charge generating layer and transporting the holes through the charge transport layer include, for example, triphenylmethane, bis(4-diethylamine-2-methylphenyl)phenylmethane; 4'-4"-bis(diethylamino)-2', 2"-dimethyltriphenylmethane, N,N'-bis(alkylphenyl)-[1,1'-biphenyl]-4,4'-diamine wherein the alkyl is, for example, methyl, ethyl, propyl, n-butyl, etc., N,N'-diphenyl-N,N'-bis(chlorophenyl)-[1,1'-biphenyl]-4,4'-diamine, N,N'-diphenyl-N,N'-bis(3"-methylphenyl)-(1,1'-biphenyl)-4,4'-diamine, and the like dispersed in an inactive resin binder.

Any suitable inactive resin binder soluble in methylene chloride or other suitable solvent may be employed in the process of this invention. Typical inactive resin binders soluble in methylene chloride include polycarbonate resin, polyester, polyarylate, polyacrylate, polyether, polysulfone, and the like. Molecular weights can vary, for example, from about 20,000 to about 1,500,000.

The preferred electrically inactive resin materials are polycarbonate resins have a molecular weight from about 20,000 to about 120,000, more preferably from about 50,000 to about 100,000. The materials most preferred as the electrically inactive resin material is poly(4,4'-dipropylidene-diphenylene carbonate) with a molecular weight of from about 35,000 to about 40,000, available as Lexan 145 from General Electric Company; poly(4,4'-isopropylidene-diphenylene carbonate) with a molecular weight of from about 40,000 to about 45,000, available as Lexan 141 from the General Electric Company; a polycarbonate resin having a molecular weight of from about 50,000 to about 100,000, available as Makrolon from Farbenfabriken Bayer A. G., a polycarbonate resin having a molecular weight of from about 20,000 to about 50,000 available as Merlon from Mobay Chemical Company and poly(4,4'-diphenyl-1,1'-cyclohexane carbonate) with a molecular weight of from about 35,000 to about 40,000, available as PCZ 400 available from Mitsubishi Chemical Co. Excellent results are achieved when the charge transport layer comprises N,N'-diphenyl-N,N'-bis(3-methylphenyl)-[1,1'-biphenyl]-4,4'-diamine in poly(4,4'-diphenyl-1,1'-cyclohexane carbonate) binder.

Examples of photosensitive members having at least two electrically operative layers include the charge generator layer and diamine containing transport layer members disclosed in U.S. Pat. No. 4,265,990, U.S. Pat. No. 4,233,384, U.S. Pat. No. 4,306,008, U.S. Pat. No. 4,439,507. The disclosures of these patents are incorporated herein in their entirety.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like. Generally, the thickness of the transport layer is between about 5 micrometers to about 100 micrometers, but thicknesses outside this range can also be used. A dried thickness of between about 18 micrometers and about 35 micrometers is preferred with optimum results being achieved with a thickness between about 20 micrometers and about 29 micrometers. Preferably, the charge transport layer comprises an arylamine small molecule dissolved or molecularly dispersed in a polycarbonate.

Other layers such as conventional ground strips comprising, for example, conductive particles disposed in a film forming binder may be applied to one edge of the photoreceptor in contact with the conductive surface or layer, blocking layer, adhesive layer or charge generating layer.

Optionally, an overcoat layer may also be utilized to improve resistance to abrasion. In some cases a back coating may be applied to the side opposite the photoreceptor to provide flatness and/or abrasion resistance. These overcoating and backcoating layers may comprise organic polymers or inorganic polymers that are electrically insulating or slightly semi-conductive.

The improved electrophotographic imaging members of this invention exhibit greater sensitivity. The donor dopant molecules of this invention containing hydroxy and methoxy substituents have lower charge carrier mobilities (resulting from the high dipole content of these substituents) than the molecules without these substituents. Therefore, they cannot be employed as charge transport molecules in the transport layer (and thereby diffuse into the generator layer) of devices required to operate in imaging machines with high print production rates per second. Without these hydroxy or methoxy substituents, however, the solubility of the donor molecules in the polyvinyl butyral binder matrix employed in the generator is very limited. Thus, this invention achieves the dual objectives of high photogeneration in the generator layer (resulting from the presence of donor molecules in the generator layer) with the molecules without these hydroxy and methoxy side groups in the transport layer achieving high mobility for the carriers injected into the transport layer. By doping the donor molecule in the generator layer, the sensitivity of the photoreceptor can be precisely tailored to satisfy extremely tight specifications even when there are batch to batch quality variations in the generator layer binder, generating layer photoconductive pigments or undercoat layer polymer.

#### PREFERRED EMBODIMENT OF THE INVENTION

The invention will now be described in detail with respect to the specific preferred embodiments thereof, it being understood that these examples are intended to be illustrative only and that the invention is not intended to be limited to the materials, conditions, process parameters and the like recited herein. All parts and percentages are by weight unless otherwise indicated.

#### ELECTRICAL SCANNING TEST

The electrical properties of photoconductive imaging samples prepared according to Examples I, II, III and IV were evaluated with a xerographic testing scanner comprising a cylindrical photoreceptor drum having a diameter of 8.4 cm. When rotated, the drum produced a constant surface speed of 7.4 cm per second. A direct current pin corotron, exposure light, erase light, and three electrometer probes were mounted around the periphery of the photoreceptor samples. The sample charging time was 33 milliseconds. Both expose and erase lights were red LED bars with output wavelength at 660 nm. The output energy of the LED bar was controlled by varying the applied voltage to the LED bar. The relative locations of the probes and lights are indicated in the Table below:

TABLE

| Element | Angle (Degrees) |
|---------|-----------------|
| Charge  | 0               |
| Probe 1 | 14              |
| Expose  | 30              |

TABLE-continued

| Element | Angle<br>(Degrees) |
|---------|--------------------|
| Probe 2 | 90                 |
| Erase   | 225                |
| Probe 3 | 345                |

The test samples were first rested in the dark for at least 60 minutes to ensure achievement of equilibrium with the testing conditions at 35 percent relative humidity and 20° C. Each sample was then negatively charged in the dark to a development potential of about 700 volts. The charge acceptance of each sample and its residual potential after discharge by front erase exposure to 400 ergs/cm<sup>2</sup> were recorded. The test procedure was repeated to determine the photoinduced discharge characteristic (PIDC) of each sample by exposing the photoreceptor device to different light energies of up to 20 ergs/cm<sup>2</sup>.

#### COMPARATIVE EXAMPLE I

A charge blocking layer was fabricated from a 14.4 percent by weight solution of zirconium butoxide and gamma-amino propyl tri-methoxy silane in an isopropyl alcohol, butyl alcohol and water mixture. The isopropyl alcohol, butyl alcohol and water mixture proportions were 66, 33 and 1 percent by weight, respectively, based on the combined weight of the isopropyl alcohol, butyl alcohol and water. The zirconium butoxide and gamma-amino propyl tri-methoxy silane mixture percentages were 90 and 10 percent by weight, based on the combined weight of the zirconium butoxide and gamma-amino propyl tri-methoxy silane. The charge blocking layer was dip coated onto an aluminum drum substrate and dried at a temperature of 130° C. for 20 minutes. The dried zirconium silane film had a thickness of about 0.1 micrometer. A charge generation coating dispersion was prepared by dispersing 22 grams of benzimidazole perylene particles having an average particle size of about 0.4 micrometer into a solution of 10 grams polyvinyl butyral (B-79, available from Monsanto Chemical Co.) dissolved in 368 grams of n-butyl acetate solvent. This dispersion was milled in a Dymonill mill (KDL, available from GlenMill) with zirconium balls having a diameter of 0.4 millimeter for 4 hours. The average particle size of the benzimidazole perylene pigment particles in the dispersion after the milling was about 0.1 micrometer. The drum with the charge blocking layer coating was dipped in the charge generation coating dispersion and withdrawn at a rate of 20 centimeters per minute. The resulting coated drum was air dried to form a 0.5 micrometer thick charge generating layer. A charge transport layer coating solution was prepared containing 40 grams of N,N'-diphenyl-N,N'-bis(3-methylphenyl)-[1,1'-biphenyl]-4,4'-diamine and 60 grams of poly(4,4'-diphenyl-1,1'-cyclohexane carbonate) (PCZ 400 available from Mitsubishi Chemical Co.) dissolved in a solvent mixture containing 80 grams of monochlorobenzene and 320 grams of tetrahydrofuran. The charge transport coating solution was applied onto the coated drum by dipping the drum into the charge transport coating solution and withdrawing at a rate of 150 centimeters per second. The coated drum was dried at 110° C. for 20 minutes to form a 20 micrometer thick charge transport layer. The resulting photoreceptor drum was electrically cycled in a scanner in a controlled atmosphere of 35 percent relative humidity and 20° C. The scanner is described above.

#### COMPARATIVE EXAMPLE II

The process described in Example I was repeated except that the charge generation layer dispersion used for coating

was different. The charge generation layer dispersion was prepared as described in the Example I, but was modified by the addition of 2.2 gram of N,N'-diphenyl-N,N'-bis(3-methylphenyl)-[1,1'-biphenyl]-4,4'-diamine (TPD) after the milling. The TPD is not compatible with the polyvinyl butyral binder. The dried film containing only polyvinyl butyral and TPD is translucent, an indication of incompatibility. When the resulting photoreceptor drum was electrically cycled in a scanner under the same conditions as described in Example I, there was no improvement on sensitivity with this charge generation layer dispersion.

#### EXAMPLE III

The process described in Example I was repeated except that the charge generation layer dispersion used for coating was different. A charge generation layer dispersion was prepared as described in the Example I, but was modified by the addition of 2.2 grams of N,N'-diphenyl-N,N'-bis(3-hydroxyphenyl)-[1,1'-biphenyl]-4,4'-diamine (DHTBD) after the milling. The DHTBD is compatible with the polyvinyl butyral binder. The dried film containing only polyvinyl butyral and DHTBD is transparent, an indication of compatibility. The resulting photoreceptor drum was electrically cycled in a scanner under the same conditions as described in Example I. The sensitivity was improved by lowering the surface voltage at the PIDC tail, evident as a lower voltage reading at 9 ergs/cm<sup>2</sup> exposure energy as compared to the readings for Examples I and II.

#### EXAMPLE IV

The process described in Example I was repeated except that the charge generation layer dispersion used for coating was different. A charge generation layer dispersion was prepared as described in the Example I, but was modified by the addition of 2.2 grams of N,N'-di(3-methoxyphenyl)-N,N'-diphenyl-[1,1 biphenyl]-4,4'-diamine (DMTBD) after the milling. The dried film containing only polyvinyl butyral and DMTBD is transparent, an indication of compatibility. The resulting photoreceptor drum was electrically cycled in a scanner under the same conditions as described in Example I. The sensitivity was improved by lowering the surface voltage at the PIDC tail, evident as a lower voltage reading at 9 ergs/cm<sup>2</sup> exposure energy as compared to the readings for Examples I and II.

The results of the scanner tests are shown in the following table:

|                                | Example I | Example II | Example III | Example IV |
|--------------------------------|-----------|------------|-------------|------------|
| V <sub>depletion</sub> (Volts) | 92        | 77         | 93          | 117        |
| V <sub>H</sub>                 | 684       | 687        | 687         | 681        |
| Dark Decay (Volts)             | 24        | 22         | 22          | 25         |
| dV/dX (V.cm <sup>2</sup> /erg) | 101       | 101        | 103         | 102        |
| V (9 ergs/cm <sup>2</sup> )    | 75        | 71         | 56          | 59         |
| V <sub>t</sub> (Volts)         | 12        | 12         | 12          | 11         |

The symbols employed in the above table are defined as follows:

Dark Decay is the voltage difference between the first and second probes.

V<sub>H</sub> is the voltage measured at the first probe.

dV/dX is the initial slope of the PIDC curve.

V (9 ergs/cm<sup>2</sup>) is the voltage measured at the first probe after the photoreceptor is exposed to light of intensity 9 ergs/cm<sup>2</sup>.

## 13

$V_r$  is the voltage measured at the third probe.

## EXAMPLE V

Several charge generation coating dispersions were prepared by dispersing 22 grams of benzimidazole perylene particles having an average particle size of about 0.4 micrometer into a solution of 10 grams several polymers. These polymers included (1) polyvinyl butyral (B-79, available from Monsanto Chemical Co.) dissolved in 368 grams of n-butyl acetate solvent, (2) poly (4,4'-diphenyl-1,1'-cyclohexane carbonate) (available as PCZ400 from Mitsubishi's electric) dissolved in a solvent mixture containing 184 grams of toluene and 184 grams of tetrahydrofuran, (3) polyamide (CM8000 from Toray) dissolved in 368 grams of butanol, (4) polyester (PE-100 from Goodyear) dissolved in 368 grams of tetrahydrofuran, (4) polymethylmethacrylate (from Scientific Polymer Products, Inc.) dissolved in a solvent mixture containing 368 grams of tetrahydrofuran, and (5) cellulose acetate (from Scientific polymer products, Inc.) dissolved in 368 grams of cyclohexanone. This dispersion was milled in a dynomill mill (KDL, available from GlenMill) with zirconium balls having a diameter of 0.4 millimeter for 4 hours. The dispersion quality was checked with a particle size distribution analyzer (CAPA from Horiba). It was found that the dispersion quality was very poor in all cases except with polyvinyl butyral.

Although the invention has been described with reference to specific preferred embodiments, it is not intended to be limited thereto, rather those having ordinary skill in the art will recognize that variations and modifications may be made therein which are within the spirit of the invention and within the scope of the claims.

What is claimed is:

1. An electrophotographic imaging member comprising a supporting substrate,

a charge generating layer comprising

photoconductive pigment particles selected from the group consisting of benzimidazole perylene and dibromoanthrone,

a film forming binder comprising polyvinyl butyral and a donor charge transporting molecule dissolved in the binder, the donor charge transport molecule selected from the group consisting of N,N'-diphenyl-N,N'-bis(3-hydroxyphenyl)-[1,1'-biphenyl]-4,4'-diamine, N,N'-di(3-methoxyphenyl)-N,N'-diphenyl-[1,1'-biphenyl]-4,4'-diamine and mixtures thereof and

a charge transport layer,

the charge generating layer being located between the substrate and the charge transport layer.

2. An electrophotographic imaging member according to claim 1 wherein the charge generating layer comprises 5 percent by volume to about 90 percent by volume of the dibromoanthrone photoconductive pigment particles dispersed in about 10 percent by volume to about 95 percent by volume of the film forming binder comprising polyvinyl butyral.

3. An electrophotographic imaging member according to claim 1 wherein the charge transporting molecule in the generating layer comprises between about 5 and about 30 percent by weight of the charge transporting molecule

## 14

selected from the group consisting of N,N'-diphenyl-N,N'-bis(3-hydroxyphenyl)-[1,1'-biphenyl]-4,4'-diamine, N,N'-di(3-methoxyphenyl)-N,N'-diphenyl-[1,1'-biphenyl]-4,4'-diamine and mixtures thereof, based on the total weight of the charge generating layer.

4. An electrophotographic imaging member according to claim 1 wherein the charge transport layer comprises N,N'-diphenyl-N,N'-bis(3-methylphenyl)-[1,1'-biphenyl]-4,4'-diamine and the film forming binder in the charge generating layer comprises a polycarbonate binder.

5. An electrophotographic imaging member according to claim 4 wherein the polycarbonate film forming binder comprises poly(4,4'-diphenyl-1,1'-cyclohexane carbonate).

6. An electrophotographic imaging member according to claim 1 wherein the charge generating layer comprises 5 percent by volume to about 90 percent by volume of the benzimidazole perylene photoconductive pigment particles dispersed in about 10 percent by volume to about 95 percent by volume of the film forming binder comprising polyvinyl butyral.

7. A process for fabricating an electrophotographic imaging member comprising

forming a charge generating layer from a coating solution of comprising

photoconductive pigment particles selected from the group consisting of benzimidazole perylene and dibromoanthrone dispersed in a film forming binder,

a hole transporting small molecule selected from the group consisting of N,N'-diphenyl-N,N'-bis(3-hydroxyphenyl)-[1,1'-biphenyl]-4,4'-diamine, or N,N'-di(3-methoxyphenyl)-N,N'-diphenyl-[1,1'-biphenyl]-4,4'-diamine and mixtures thereof dissolved in the binder,

forming a charge transport layer coating comprising N,N'-diphenyl-N,N'-bis(3-methylphenyl)-[1,1'-biphenyl]-4,4'-diamine,

a polycarbonate binder and

a solvent, and

drying the coating to form a charge transport layer overlying the charge generating layer.

8. A processes for fabricating an electrophotographic imaging member according to claim 7 wherein the charge transporting molecule in the generating layer comprises between about 5 and about 30 percent by weight of the charge transporting molecule selected from the group consisting of N,N'-diphenyl-N,N'-bis(3-hydroxyphenyl)-[1,1'-biphenyl]-4,4'-diamine, N,N'-di(3-methoxyphenyl)-N,N'-diphenyl-[1,1'-biphenyl]-4,4'-diamine and mixtures thereof, based on the total weight of the charge generating layer.

9. A processes for fabricating an electrophotographic imaging member according to claim 7 wherein the polycarbonate film forming binder comprises poly(4,4'-diphenyl-1,1'-cyclohexane carbonate).

10. A processes for fabricating an electrophotographic imaging member according to claim 7 wherein the photoconductive pigment particles comprise benzimidazole perylene pigment particles.